

Aug. 18, 1936.

O. CHRISTENSON

2,051,200

## SOUND REPRODUCING DEVICE

Filed Sept. 14, 1933

2 Sheets-Sheet 1



## WITNESSES

WITNESSES

**INVENTOR**  
*Oscar Christenson*

BY

Wm. Anderson, Stanley Foster, Ladd  
ATTORNEYS

Aug. 18, 1936.

O. CHRISTENSON

2,051,200

SOUND REPRODUCING DEVICE

Filed Sept. 14, 1933

2 Sheets-Sheet 2



## WITNESSES

**WITNESSES**

INVENTOR

BY

BY  
Munro Anderson, Stanley, Foster & Ladd  
ATTORNEY

## UNITED STATES PATENT OFFICE

2,051,200

## SOUND REPRODUCING DEVICE

Oscar Christenson, Baltimore, Md.

Application September 14, 1933, Serial No. 689,459

6 Claims. (Cl. 179—110)

This invention relates to a device for producing sound.

An object of the invention is the provision of a device for the reproduction of sound and which may be employed as a loud speaker, in which a plate is employed formed of two sheets of thin metal having different co-efficients of expansion, with the sheets being secured together at a predetermined temperature so that when the plate is cooled the sheets will be under a compressive and tensile stress, such a plate being subject to changes caused by magnetostriction, a vibratory member being rigidly connected with the plate.

Another object of the invention is the provision of a sound-reproducing device based on the magnetostriction principle and adapted for use as a loud speaker unit in which a plate is subjected to changes caused by magnetostriction, a cone or other form of diaphragm being rigidly connected to the composite plate by means of a rod secured at the center of the plate so that the receiver becomes an efficient loud speaker unit.

The composite plate of the present receiver vibrates with great force and a cone or other diaphragm connected with the plate may therefore be of greater size and weight than would be practicable in the case of a dynamic or magnetic speaker. By increasing its area, thickness and rigidity the cone may be made a more efficient radiator of sound waves.

A further object of the invention is the provision of a sound reproducing device in which a plate is formed of a thin sheet of nickel secured in any approved manner to the metal plate having a thermal co-efficient of expansion which is greater than the co-efficient of the nickel, so that the nickel plate is maintained under permanent compressive stress which is utilized to increase its magnetic susceptibility and magnetostriction when varying currents are passed through the coil to place the plate for imparting to a cone or diaphragm the vibrations for the reproductions of sound waves, the plate being rigidly secured at its opposite ends to a permanent magnet employed in connection with the loud speaker unit.

This invention will be best understood from a consideration of the following detailed description, in view of the accompanying drawings forming a part of the specification; nevertheless, it is to be understood that the invention is not confined to the disclosure, being susceptible of such changes and modifications as define no material departure from the salient features of the invention as expressed in the appended claims.

## In the drawings:

Figure 1 is a view in elevation partly in section showing a sound reproducing device constructed in accordance with the principles of my invention,

Figure 2 is a view in elevation of the reproducing unit with the cover in section,

Figure 3 is a transverse vertical section of the unit shown connected to a cone,

Figure 4 is a view in elevation of the unit with the cover in section showing a modified form of the sound-reproducing device and taken along the line 4—4 of Figure 5,

Figure 5 is a section taken at right angles to the section shown in Figure 4, and

Figure 6 is a view in perspective of a permanent magnet showing the blocks for rigidly supporting the opposite ends of a plate.

Referring more particularly to the drawings, 10 designates a base member formed of insulating material or of metal, such as aluminum, and this base member is neatly fitted within one end of a cylinder 11 and connected to said cylinder, as shown at 11a.

The outer end of the cylinder is provided with a closure 12 which has a centrally disposed opening 13 through which projects a threaded rod 14. The cover may be formed integrally with the cylinder or may be made separately and connected thereto. A ring magnet 15 is secured to the base member 10 and is formed of good magnet steel permanently magnetized across the diameter in line with the pole pieces 17a. This magnet forms a polarizing field for a nickel plate which will be presently described. The magnet 15 is secured to the base member 10 in any approved manner and by means of screws 16. Blocks 17a formed of soft steel are likewise secured in position and on the inner face of the permanent magnet 15 by the screws 16.

A pair of bars 22 and 23 extend diametrically of the base member 10 with the bar 22 resting at diametrically opposite points on the magnet 15. These bars are connected together at their ends by means of bolts 24 with the bolts being screwed into threaded perforations in the bar 22. The inner portions of the bars are cut away, as shown at 21, to provide a space for a purpose which will be presently explained.

The metal plate is formed of two thin sheets of metal, such as zinc as indicated at 30, and a sheet formed of pure nickel, indicated at 31. These plates have their adjacent faces, as shown at 32, secured together by means of soldering. The nickel plate is approximately .005 of an inch

in thickness, 2 inches in width and  $2\frac{1}{2}$  inches in length while the zinc plate is approximately  $\frac{1}{8}$  of an inch in thickness, 2 inches in width and  $2\frac{1}{2}$  inches in length. Pure nickel is employed of dead soft temper. Any appreciable variation from the thickness of the nickel will result in a decrease in sensitivity of the device. The nickel plate and zinc plate are tinned on one side with solder and are pressed together with their tinned surfaces in contact between steel plates which are in turn placed between the jaws of a vice. The whole is then heated in any approved manner until the solder on the surface of the plates is melted. The plates are then pressed tightly together and allowed to cool before removal from the vice. Any metal, alloy, or material having a linear coefficient of expansion greater than that of nickel may be used to subject the nickel plate to a permanent compressive stress and among such metals having the largest coefficients of expansion are zinc, aluminum, lead, tin, and porcelain. However, lead and tin give results which are far below those obtained from zinc due to their low melting points and low tensile strength. It has been found, however, that aluminum, and especially zinc, give the best results. The zinc plate soldered to the nickel plate, the solder having a melting point of approximately  $450^{\circ}$  Fr., will subject the nickel to a degree of compressive stress in which condition its susceptibility and magnetostrictive effects are greatest.

A form 40 made of bakelite or of other rigid insulating material has wound thereon coils of wire 45 and 46. These coils are provided in the form of a winding of No. 40 B & S gage enamel insulated copper wire. Both coils are wound in the same direction, each coil being simply a continuation of the other. In winding the following procedure is followed: The assembly is placed in the winding machine and the end of the wire from the spool supply is passed through an opening in one of the bars 22 or 23 and temporarily secured in place. The wire is then wrapped around one section upon one side of the bars 22 and 23 until this section is secured. The assembly is then turned around in the winding machine so that it will revolve in the opposite direction. The end of the wire from the spool supply is joined to that end of the first coil which was temporarily secured in place before commencing the winding. The remaining section is then filled with the winding. This construction has the advantage that both terminals of the winding are brought out at the upper surface of the winding. One terminal 49 is connected as shown to a metal plate 50 held in position by the screw 24. The other terminal 51 of the winding is connected to a metal plate 52 held in place by the screw 24. A wire 53 is connected to the metal plate 50 while a wire 54 is connected to the plate 52. The wires 53 and 54 are the lead-in wires from the instrument.

A sheet of insulating material may be wound around the exterior of the coils 45 and 46 and cemented in position if desired by a suitable lacquer.

The plate formed of the thin sheets of zinc and nickel are rigidly secured at their opposite ends to the steel blocks 17 preferably with the nickel surface in contact with the steel blocks and these blocks are connected to the permanent magnet 15.

The rod 14 has its inner end connected to the metal plate by means of a head 61 and nuts 62 and 63.

A diaphragm or cone which constitutes a vibrating element for the reproduction of a sound is shown at 65 and this cone is connected to the outer free end 66 of the rod 60. Metal plates 67 and 68 are located upon opposite sides of the diaphragm and are held in place by nuts 69 and 70 threaded onto the rod and into close contact with the plates 68 and 67, respectively.

The purest nickel obtainable annealed to the softest temper is employed in the manufacture of the plate 31. It is to be noted that the removal of harmful impurities from the nickel and annealing it to the softest temper greatly increases the permeability and magnetostrictive effect and thereby the sensitivity of the speaker unit. 15

The loud speaker unit may be connected in the output circuit of a vacuum tube or coupling transformer or in any other desired way. For best results the magnetizing coils of the speaker unit should be wound to match or slightly ex- 20 ceed the impedance of the output circuit.

This loud speaker unit operating in connection with a cone diaphragm placed in a baffle of standard dimensions gives high quality reproduction of speech and music in ample volume with power 25 input no greater than that required by standard types of speakers in wide commercial use.

Owing to its light weight and the great rigidity with which the vibratory plate is supported it is especially suited for installation in automobiles 30 and airplanes where severe vibration occurs.

In my pending application S. N. 611,411 I have stated that the telephone receiver described therein operates by changes in the thickness of the nickel or other magnetostrictive metal or 35 alloy in the composite plate. It is probable that such changes in thickness of the plate occurs. Changes in thickness of only a small fraction of a millionth of an inch would be sufficient to set up an audible sound wave. With the minute currents necessary to actuate the receiver it is quite possible it may operate in this way. 40

Much greater power is required to operate the loud speaker unit and there can be no doubt that in the present construction the composite plate 45 vibrates in a flexural manner. Nickel contracts in the direction of a magnetic field and expands perpendicularly in fields of all intensities apparently tending to a fixed limit as the magnetizing force is raised to high values. The audio currents in the magnetizing coils surrounding the composite plate set up a varying magnetic field and cause proportional magnetostrictive contractions in the thin nickel sheet which flexes the composite plate as a whole which in turn 55 transmits its vibrations to the cone diaphragm.

The zinc plate used in constructing the composite plate is of a thickness sufficient to give the structure a frequency responsive characteristic well up in the audible range. If it is desired to 60 raise still further the natural frequency of vibration of the composite plate its zinc component may be increased to double or more its present thickness with but slight decrease resulting in the sensitivity of the loud speaker unit. In all 65 types of telephone receivers in commercial use at the present time of which I have any knowledge the diaphragm is actuated by forces from outside of itself. If such diaphragms are increased in size beyond a definite limit they be- 70 come extremely inefficient.

In the present construction employing the composite plate or diaphragm the plate is actuated by magnetostrictive forces within the plate itself. If the plate is supplied with enough power the 75

magnitude of these forces increase as the size of the plate is increased.

A composite plate to act as the vibratory element in the loud speaker may be constructed so that its magnetostrictive component will be under tensile stress. It has been found that the magnetic susceptibility and magnetostriction effects are increased in some metals and alloys such as some of the nickel-iron alloys more by tensile stress than by compressive stress. The alloy Invar has one of the smallest coefficients of expansion known.

If a sheet of Invar is secured by soldering, brazing or welding to a sheet of almost any other metal or alloy it will result in setting up permanent tensile stress in the other metal or alloy.

I have constructed a number of such composite plates in which the magnetostrictive sheet is under tension using plates of Invar with thin sheets of Platinite and other iron-nickel alloys but as vibratory elements for use in telephone receivers and loud speakers I have found them less sensitive than the composite plate constructed of zinc and nickel.

The polarizing field required on the composite plate of the loud speaker unit and of the telephone receiver is critical as to intensity. If the polarizing field is of too great intensity it reduces the sensitivity of the device. The ring magnet described is designed to supply a polarizing field to the plate of an intensity at which its sensitivity is the greatest. If the magnet establishes too strong a field on the plate the polarizing field may be decreased by inserting a shim of brass or of other non-magnetic material between the pole pieces on the magnet and the composite plate.

The polarizing field may be made adjustable by methods well known in the art such as varying the distance between the permanent magnet and the composite plate by means of an adjusting screw operating on the magnet. When the speaker unit is connected in the output circuit of a vacuum tube the steady component of the vacuum tube plate current through the coils surrounding the composite plate may establish sufficient magnetism in the plate to maintain the speaker unit at its maximum sensitivity without the aid of a permanent magnet.

The necessary polarizing field may be supplied by means of an auxiliary coil or coils wound around the composite plate and connected with a source of direct current supply. The direct current supply on the other hand may be connected to the coils surrounding the composite plate carrying the audio currents and choke coils of suitable inductance inserted in the direct current supply circuit to prevent the short circuiting of the audio currents.

A plate 31<sup>a</sup> which is formed of pure nickel of medium hard temper approximately .02 of an inch thick, 2 inches wide and of such a length that when it is forced down by means of screws to its seat on the steel blocks 17<sup>a</sup> carrying the projecting wedges 81 shown in Fig. 6 it will be under a degree of compression at which its magnetic susceptibility and magnetostriction effect are greatest, may be used in place of the composite plates described. This method, however, of setting up compressive stress in the nickel plate is not as effective as the differential thermal contraction method and as a vibratory element for use in telephone receivers and loud speakers the pure nickel plate is not as efficient as the nickel-zinc composite plate.

A thin sheet of nickel, platinite or other high-

ly magnetostrictive metal or alloy cemented with gytal varnish or otherwise firmly secured to a somewhat thicker sheet of stiff material such as bakelite or hard rubber may be substituted for the composite plate in a telephone receiver. The magnetostrictive metal in this case is not under compressive or tensile stress.

The composite plates may be made in large sizes for use in loud speakers without cones or other radiating members being attached thereto. These plates as thus constructed are operated as direct radiators of sound. It will be appreciated, however, that sufficient power will have to be applied to operate these larger plates. Soft rubber washers 100 which are unusually thin are inserted under the heads of the screws 24 and between the nickel surface of the composite plate which is firmly clamped between the soft rubber washers. Such construction decidedly improves the performance of the device. The soft rubber washers tend also to prevent the vibrations of the plate from being transmitted to the casing or other parts of the assembly.

I claim:—

1. In a sound reproducing device, a plate formed of magnetostrictive metal which is under compressive stress, means coacting with the opposite ends of said plate for maintaining the plate under compressive stress, a coil of wire adjacent the plate adapted to have a current passed therethrough to set up a varying magnetic field, means for maintaining the plate in a magnetized state, and a diaphragm connected with the plate.

2. In a sound reproducing device, a plate formed of two sheets of metal rigidly secured together, one of the sheets being formed of magnetostrictive metal, one of the sheets being under tensile stress, means coacting with the opposite ends of the plate for maintaining the plate under compressive stress, a coil of wire adjacent the plate adapted to have a current passed therethrough to set up a varying magnetic field, means for maintaining the plate in a magnetized state, and a diaphragm connected with the plate.

3. In a sound reproducing device, a plate formed of magnetostrictive metal which is under compressive stress, means coacting with the opposite ends of said plate for maintaining the plate under compressive stress, a coil of wire adjacent the plate adapted to have a current passed therethrough to set up a varying magnetic field, means for maintaining the plate in a magnetized state, a diaphragm connected with the plate, and means for cushioning the ends of the plate.

4. In a sound reproducing device, a plate formed of two sheets of metal rigidly secured together, one of the sheets being formed of magnetostrictive metal, one of the sheets being under compressive stress, the other sheet being under tensile stress, means for securing the opposite ends of the plate in position, a coil of wire adjacent the plate adapted to have a current passed therethrough to set up a varying magnetic field, means for maintaining the plate in a magnetized state, a diaphragm connected with the plate, and means for cushioning the ends of the plate.

5. In a sound reproducing device, a plate having magnetostrictive metal applied thereto which is under a compressive stress, means coacting with the opposite ends of the plate for maintaining the plate under compressive stress,

a coil of wire adjacent the plate adapted to have a current passed therethrough to set up a varying magnetic field, means for maintaining the plate in a magnetized state, a rod rigidly connected at one end with the center of the plate, and a diaphragm connected with the free end of the rod.

6. In a sound reproducing device, a plate formed of two sheets of metal, one of the sheets being formed of magnetostrictive metal, said sheets being secured together at a high tem-

perature and respectively being under compressive and tensile stresses so that a permanent compressive stress and a permanent tensile stress are set up in the plate when the secured sheets have been cooled, a magnet, means for securely fastening the ends of the plate to the magnet, a coil adjacent the plate adapted to have varying currents passed therethrough, and a diaphragm rigidly connected with the plate. 5

10

OSCAR CHRISTENSON.